

# UNITED STATES PATENT OFFICE.

PAUL RAKOWICZ, OF GRIESHEIM, GERMANY, ASSIGNOR TO THE FIRM OF CHEMISCHE FABRIK GRIESHEIM-ELEKTRON, OF FRANKFORT-ON-THE-MAIN, GERMANY.

## PREPARATION OF IRON OR STEEL FOR CASTING.

No. 927,678.

Specification of Letters Patent.

Patented July 13, 1909.

Application filed November 18, 1908. Serial No. 463,303.

To all whom it may concern:

Be it known that I, PAUL RAKOWICZ, a subject of the German Emperor, and resident of Griesheim-on-the-Main, Germany, 5 have invented certain new and useful Improvements in Connection with the Preparation of iron or Steel for Castings, of which the following is a specification.

Magnesium used in the manufacture of 10 iron, and steel, for casting, greatly improves the castings, as it makes them dense and free from blow-holes, imparts to them a homogeneous structure and greatly advances their physical properties. Magnesium acts in 15 this connection much better than aluminium, and the use of magnesium in making iron and steel for castings has been before proposed and has formed the subject of many patents, but its use as a deoxidizing agent 20 has not hitherto been industrially successful in making iron and steel for casting as its addition to molten iron, or steel, has been exceedingly difficult, very violent action taking place, and the molten metal being projected out of the receptacle, and therefore 25 the addition of magnesium to molten iron, or steel, in the same manner as is practiced with aluminium, is unsuitable for practical purposes.

30 In the specification of the German Patent 86,607, dated March 5, 1895, it is proposed to use, for deoxidizing iron, and steel, alloys of aluminium, or of alkaline earth metals, such as magnesium, with iron and non 35 metals, such as silicon, and boron, which form slags. The specification of the said patent does not however describe any way of preparing, for the purpose, an alloy, containing magnesium.

40 Another proposal for avoiding the violent action which takes place on the addition of magnesium to molten iron, or steel, is described in the specification of the Swedish Patent No. 261 of the 8th February A. D. 45 1905 and consists in the supply of gaseous magnesium to the iron, or steel. This mode is however not without danger and it is very troublesome and does not afford any guarantee that the deoxidization will be 50 properly carried out.

This invention provides a process of working which is free from danger, and which can be applied to heavy charges with efficiency and ease.

I have found that the magnesium should 55 be introduced into the iron, or steel, when the latter metal forms a semifluid or thickly liquid mass in passing from the solid to the fluid state. When the steel, or iron, is in this thick condition, the introduction of the 60 magnesium takes place smoothly. As it is not convenient in the manufacture of iron and steel for casting to cool the melt to such an extent that the magnesium can be introduced therewith safety, a preliminary 65 alloy is formed, which is added in a thick state, or in a liquid state, to the iron, or steel, to be deoxidized and cast in the same manner as other additions are made, such, for instance, as aluminium, ferro-silicon, or ferro-manganese. Iron and steel have but little affinity for magnesium and in this respect act in a manner the opposite to that of copper, nickel, or the like, but it is possible to obtain in the aforesaid manner a ferro-magnesium containing a small percentage of magnesium.

The alloy may be formed in several ways. For instance, a suitable quantity of iron or steel is heated to such a degree that it becomes semi-fluid, and then a block of magnesium is introduced into the thick liquid and unites therewith. The block may be introduced by fixing it to the end of an iron rod having a protecting coating of clay or similar 80 material. The magnesium may be in the form of a cup-shaped block having a perforation into which one end of the rod may be inserted.

In order to fully deoxidize 100 kilograms 90 of iron, or steel, for casting, from 15, to 50, grams of magnesium are required according to the quality of the iron, or steel, used. It is therefore necessary to add to 100 kilograms of iron, or steel, for casting from 1.5, to 5, 95 kilograms of a preliminary alloy containing 1 per cent. of magnesium. If additions of other metal such as nickel, or aluminium, are also to be made to the iron, or steel, these can, if desired, be introduced into the preliminary alloy, the said additions being, for instance, first alloyed with magnesium and this alloy being introduced into the iron, or steel for the production of the preliminary alloy.

I claim:

1. The method of alloying iron or steel with magnesium which consists in first pass-

ing iron or steel from the solid into a semi-fluid or thickly liquid state then introducing magnesium into the thick mass, as and for the purpose set forth.

5 2. The method of deoxidizing iron or steel by first passing a quantity of iron or steel to a semifluid or thickly liquid condition, then introducing magnesium into the thick mass and then adding the alloy thus formed to the

iron or steel to be deoxidized as and for the 10 purpose set forth.

In testimony whereof I have signed my name to this specification in the presence of two subscribing witnesses.

PAUL RAKOWICZ.

Witnesses:

FRANZ HAFSLACHER,  
ERWIN DIPPEL.